

# UNITED STATES PATENT OFFICE.

FREDERICK GREENING, OF UXBRIDGE, COUNTY OF MIDDLESEX, ENGLAND,  
ASSIGNOR TO HIMSELF AND JOHN FROST, OF SAME PLACE.

## PROCESS OF PRODUCTION OF MATERIAL AS SUBSTITUTE FOR INDIA-RUBBER, &c.

### SPECIFICATION forming part of Letters Patent No. 401,269, dated April 9, 1889.

Application filed June 28, 1887. Serial No. 242,786. (No specimens.) Patented in England June 26, 1886, No. 8,442; in France June 15, 1887, No. 184,247, and in Belgium June 20, 1887, No. 77,879.

*To all whom it may concern:*

Be it known that I, FREDERICK GREENING, a subject of the Queen of Great Britain and Ireland, residing at Uxbridge, in the county 5 of Middlesex, England, have invented a new or Improved Process of Production of Material that can be used as or in the Making of Substitutes for India-Rubber, Varnish, Ivory, Whalebone, and other Substances, (for which

10 I have obtained Letters Patent as follows: In Great Britain, June 26, 1886, No. 8,442; in France June 15, 1887, No. 184,247, and in Belgium June 20, 1887, No. 77,879, the said patents of France and Belgium being in the 15 name of Frederick Greening and John Frost,) of which the following is a specification.

This invention relates to a new or improved manufacture of material that can be used as or in the production of substitutes for india- 20 rubber, gutta-percha, ivory, whalebone, varnish, or coating for protecting oil-paintings, water-color drawings, &c., for coating and preserving eggs, for waterproofing, capsuling, or covering, or for coating metals or wood, or as 25 a substitute for oil in mixing colors, and for other purposes.

In the manufacture of material such as "celluloid" it has heretofore been usual, in the preparation of the base, to use a mixture 30 of nitric and sulphuric acids, thus rendering the product explosive and dangerous to manufacture and use, besides necessitating the employment of expensive solvents—such as sulphuric ether, camphor, and others—for effecting the reduction of the base either to a 35 plastic mass or a solution.

Now this invention has for its object to produce a material that may be employed in lieu of celluloid, and for purposes such as above 40 indicated, and which shall be of a less explosive and less dangerous nature and can be manufactured without the use of expensive solvents such as referred to above.

In carrying out this invention fibrous substance of any suitable kind—such as paper, old rags, grass, cotton, &c.—is treated by steeping or saturating with a mixture of sulphuric acid and nitrate of potash. Suitable proportions are, say, three parts, by weight, of sul-

phuric acid (specific gravity 1.840) to two 50 parts, by weight, of nitrate of potash. When the sulphuric acid and nitrate of potash have been thoroughly incorporated and allowed to settle, the mixture is heated (for example, by hot water circulating in the jacket of a jacked pan or in a coil) to a temperature of, say, about from 75° to 90° Fahrenheit. The mixture being in this state, the fiber is now immersed in it and is thoroughly saturated. The immersion is continued and the temperature is maintained for, say, from twenty to twenty-four hours, or until it is found that the conversion has taken place. The converted fiber is then freed from excess of the mixture by pressure or otherwise, is well 60 washed with water, and is dried sufficiently to be submitted to a suitable bath for neutralizing or counteracting the effect of any trace of free acid remaining. I prefer, however, in practice to subject the converted 70 fiber to a bath of liquid carbonic acid or of carbonic-acid gas, as the material obtained by dissolving the said fiber or soluble base in a solvent is transparent, while if the fiber is treated with an alkali the resulting product is opaque or translucent. The fibrous 75 mass is to be thoroughly impregnated with the carbonic acid and afterward allowed to dry. When dry, it will be ready to be treated with a suitable solvent or solvents.

A suitable solvent is produced as follows: To one hundred gallons of methylated alcohol are added, say, from twenty-five to fifty pounds weight of refined rosin or colophony; also, from ten to twelve pounds weight of gum 85 benzoin or benjamin, and from eighty to one hundred pounds of castor-oil. The whole is thoroughly mixed and afterward distilled gradually in a still or retort until the temperature reaches, say, from 300° to 320° Fahrenheit. The distillate thus obtained is dried by any suitable means. It may be by redistilling over anhydrous lime or calcium chloride, to which, if required, there may be added some light hydrocarbon, either from the coal-tar series (such as benzole or coal-tar naphtha) or from the wood series (such as woodtar); or the hydrocarbon may be added to the 90 95

mixture of substances before effecting the first distillation, or to the solvent obtained by the second distillation. The proportion of hydro-carbon added may vary considerably. Proportions varying from ten per cent. to fifty per cent. of the weight of the mixture of substances hereinbefore specified (from which the solvent is distilled) have been found to give satisfactory results. The addition of hydro-carbon serves to counteract the tendency of the solvent to absorb moisture from the air.

The base, obtained as hereinbefore described, is dissolved in the solvent and forms a quick-drying mass or solution. It is treated or used as follows: When the material or base is to be used as a substitute for india-rubber, ivory, whalebone, and the like, it is mixed with or dissolved in a suitable proportion of solvent, so as to form a thick plastic mass, which is passed between heated rolls, whereby the material is dried and formed into hard flexible sheets, ready for use. A suitable temperature to which to heat the rolls is, say, about 100° Fahrenheit.

The material may be made of any desired color by the addition of suitable coloring agents to the plastic mass. For instance, coloring agents—such as aniline dyes or the ordinary pigments—may be used in proportions that may be varied in accordance with the tint or the density desired to be given to the finished material.

When the dissolved material or base is to be used as a varnish or coating for protecting or preserving purposes, as hereinbefore mentioned, the proportion of solvent used is such as to form a thin solution, which may be applied in any suitable way to the articles or substances to be coated. Thus for coating paintings or metals for waterproofing and the like the solution may be applied in any suitable way. It may be by a brush. For coating eggs, capsuling bottles, and the like, simple immersion of the egg or of the mouth end of the bottle-neck with its contained cork or stopper is sufficient, the coating of solution (in each case) rapidly drying after withdrawal from the bath, and so forming an efficient protective covering.

The product remaining in the still or retort after the first hereinbefore-mentioned distillation is suitable for waterproofing or for mixing with the prepared base hereinbefore described. For this purpose it is thinned down to any desired consistency by the addition of the solvent and is applied as before. This forms a good protective coating substance or solution that may, in some cases, be used as a priming-coat to an object, to be afterward

coated with a solution of the base only in the 60 solvent.

I am aware that it is old to prepare soluble cotton by soaking the same in a mixture of nitric and sulphuric acids, then washing out the traces of acid by an alkaline solution, and then drying the product; but

What I claim is—

1. The herein-described process of producing from fibrous substance a soluble base, consisting in steeping or saturating the said fibrous substance in a mixture of sulphuric acid and nitrate of potash, washing the converted fiber, then subjecting the same to a bath of liquid carbonic acid or ~~carbonic-acid~~ 70 gas, and then drying the converted fiber, substantially as described.

2. The process of treating fibrous substances, consisting of steeping or saturating said substances with a mixture of sulphuric acid and nitrate of potash, washing the converted fiber, then subjecting the same to a bath of liquid carbonic acid or carbonic-acid gas, then subjecting the same to an acid bath, then drying the converted fiber, and then treating the same with a suitable solvent, as 85 herein described.

3. The process of treating fibrous substances, consisting of subjecting the same to a mixture of sulphuric acid and nitrate of potash, washing the converted fiber, subjecting the same to a bath of liquid carbonic acid or carbonic-acid gas, then drying the converted fiber, and then treating the same with a solvent composed of a mixture of methylated alcohol, rosin, or colophony, gum benzoin 95 or benjamin, and castor-oil, substantially as described.

4. The process of treating fibrous substances with a heated mixture of sulphuric acid and nitrate of potash, then freeing the converted fiber from excess of the mixture, washing it with water, partially drying it, subjecting it to a bath of liquid carbonic acid or of carbonic-acid gas, then drying it, then treating it with a distillate composed of a mixture 105 of methylated alcohol, rosin, or colophony, gum benzoin or benjamin, castor-oil, and light hydrocarbon, substantially as herein set forth.

In testimony whereof I have signed my 110 name to this specification in the presence of two subscribing witnesses.

FREDERICK GREENING.

Witnesses:

W. LLOYD WISE,  
Patent Agent, London.

F. J. BROUGHAM,  
46 Lincoln's Inn Fields, London, W. C.